

Patented Oct. 12, 1926.

1,602,577

# UNITED STATES PATENT OFFICE.

HERBERT D. HECKERT, OF BIRMINGHAM, ALABAMA.

## PROCESS OF PRESERVING WOOD.

No Drawing.

Application filed May 6, 1925. Serial No. 28,501.

The present invention relates to the preservation of wood in the form for example of poles, piling, railway ties, blocks and yellow pine timber of various kinds, and the object of the invention is to provide a novel and improved process whereby the penetration of the preservative into the sap wood to the heart wood in the material treated may be effected more thoroughly and with less amount of preservative than has been possible with such processes as have been heretofore used or proposed.

Heretofore it has been proposed to fill the cells of the wood with creosote oil or liquid preservative by submitting the wood directly to the preservative under pressure, but such treatment would be unsuccessful commercially, as the high pressure that would be required to effect a thorough penetration of the sap wood of the material treated, or penetration of the preservative to the heart wood would involve the loss of an excessive amount of the preservative because of the highly absorptive properties of the sap wood, and any effort to avoid the loss of an excessive amount of preservative by using a lower pressure would be unsatisfactory as the oil would only partially penetrate the sap wood thus leaving portions thereof untreated or insufficiently treated and hence subject to decay or deterioration, and the relatively low pressure of the preservative in the presence of the highly absorptive properties of the sap wood would be insufficient to insure penetration of the oil to the heart wood. In other processes, heretofore used or proposed, the preservative oil injected into the wood has been permitted to remain therein for the purpose of filling the cells thereof, but such a procedure involved the consumption or loss of an excessive amount of oil or preservative.

The present invention provides a process whereby thorough penetration of the preservative oil throughout the sap wood is attained without excessive absorption of oil or preservative, so that the sap wood will be thoroughly preserved by the use of a minimum amount of oil and the avoidance of excessive absorption of the preservative oil in the sap wood enables a sufficiently high oil pressure to be applied to the wood to insure penetration of the oil to the heart wood. Moreover, the process provided by the present invention enables a substantial amount of the preservative oil employed to

be removed and recovered from the wood without impairing the preservation thereof, so that the oil thus recovered may be used in a subsequent treatment of the wood which may be effected in order to seal the cells of the wood and thus prevent loss of the preservative oil injected by the previous treatment, by leaching or evaporation.

The procedure preferably followed in treating wood for the preservation thereof by the process provided by the present invention, which may be carried out with the aid of apparatus such as that commonly used in the creosoting of wood as heretofore practiced, is substantially as follows:

The charge of wood in the form of poles, piling, ties, blocks or timber is placed in a chamber such for example as the cylinder commonly used in the creosoting of wood by other processes, and the wood is seasoned or dried, preferably by steaming in the cylinder, followed by the application of a vacuum pressure within the cylinder as is usually performed as a preliminary step in the creosoting of wood by other well known processes. This preliminary treatment, or any equivalent thereof, is for the purpose of drying the wood as thoroughly as possible and thus preparing the wood to take up the preservative oil freely and to facilitate the penetration of the oil through the sap wood.

After the wood has been thus treated in the cylinder, it is subjected to the action of an atmosphere of a gaseous medium produced for example by forcing air into the cylinder until it reaches a pressure of from 40 to 50 pounds per square inch, and while the wood is maintained under the influence of this compressed air, or without releasing the air pressure, the cylinder containing the charge of wood under treatment is pumped full of creosote oil such as that commonly used in other well known creosoting processes, or any other suitable preservative in liquid form, until the creosote oil or preservative reaches a pressure preferably of at least 150 pounds per square inch. The charge of wood is maintained under the penetrating influence of the creosote oil or preservative which submerges it substantially at the pressure thereof as stated, until about 80 per cent of the total amount of creosote oil which the wood is to receive has penetrated the wood, this being for example calculated according to the cubic feet

- of wood composing the charge under treatment, and the drop in the level of the oil in the treating tank due to the penetration of the oil into the wood, as indicated by a 5 gauge which may be provided on the treating tank. Creosote oil is preferably used as the preservative, and it is introduced into the treating cylinder at a temperature preferably of about 190° to 200° F.
- 10 After the wood has received the desired amount of creosote oil or preservative under the treatment described, the creosote oil is drawn off from the cylinder when it may be suitably stored for subsequent use, and a 15 vacuum of about 15 inches of mercury is created within the cylinder containing the wood under treatment. The purpose and effect of this vacuum treatment is to remove all excess air from the wood, and which if 20 present would resist or impede the subsequent injection of creosote oil, to be presently described, and to remove with the air any surplus oil or preservative, this vacuum treatment of the wood being continued for a 25 period preferably of at least 20 minutes.
- Upon completion of the vacuum treatment, the treating cylinder containing the wood under treatment is again filled with creosote oil, preferably at a temperature of 30 190° to 200° F. and pressure is applied to the oil until it reaches a pressure preferably of at least 110 lbs. per square inch, and this pressure is maintained until a gauge reading of the treating tank shows that the wood 35 under treatment in the cylinder and which is submerged in the body of creosote oil therein has absorbed the remaining proportion of the total amount or charge of oil which it was intended the wood should receive, 40 which would be 20 per cent of the total charge when 80 per cent of the total charge was absorbed by the first treatment described above, allowing for the amount of oil which is absorbed by the wood while the cylinder 45 is being filled with oil. The purposes and effects of this second or subsequent oil injection are to refill the cells of the wood which were emptied of oil and air by the vacuum treatment following the first oil injection, to seal the cells and thus exclude 50 moisture, fungi and germs which might cause decay of the wood, and to prevent the loss of the creosote or preservative oil by leaching or evaporation.
- 55 By submitting the wood to an atmosphere of a gaseous medium such as compressed air, and applying the oil under pressure without releasing the pressure on the air or gaseous medium, the minute cells or crevices 60 of the sap wood on the poles, ties, blocks or other bodies of wood under treatment become filled with such air or gaseous medium and hence the highly absorptive properties of the sap wood are counteracted 65 to a substantial degree, so that the oil may

be subjected to a high pressure which will insure its penetration throughout the sap wood without excessive loss of oil due to the highly absorptive properties of the sap wood and the use of a high pressure on the oil which is thus made possible enables the oil to reach into and penetrate to the heart wood. Penetration of the preservative oil throughout the sap wood and to the heart wood is thus attained by the use of a minimum amount of oil or preservative, as the loss of oil due to the highly absorptive properties of the sap wood is reduced to a minimum by reason of the presence of the air therein at the time the preservative oil is injected.

The vacuum treatment which follows the first oil injection removes any air remaining in the wood and it also removes from the wood any surplus or unabsorbed oil which will be carried or forced out of the wood with or in advance of the escaping air, thus further economizing the amount of oil used.

The subsequent or final injection of the creosote oil or liquid preservative may be accomplished at a pressure less than that employed during the preceding oil injection, as its purpose is to fill the cells of the wood which were emptied by the vacuum treatment following the first oil injection, thus protecting the wood against the entrance of moisture, fungi, germs or other destructive media, and the cells are sealed so that loss of oil by evaporation or leaching is minimized or prevented.

The wood preserving process provided by the present invention enables poles, piling, ties, blocks and other pieces of wood comprising more or less sap wood to be thoroughly treated with creosote oil or other liquid preservative with the use of a minimum amount of oil or preservative, the highly absorptive sap wood being prevented, by the air filling it during the first treatment, from taking up an excessive amount of the oil or preservative, so that a sufficiently high pressure may be applied to the preservative oil to insure its penetration into and throughout the sap wood and to the heart wood.

I claim:

1. The process of preserving wood which comprises submitting the wood to a gaseous atmosphere at a pressure above atmospheric pressure, submitting the wood to the action of a liquid preservative at a pressure substantially above that of the gaseous atmosphere, thereby coating the walls of the interior cells of the wood with the preservative, removing the gaseous atmosphere and surplus preservative from the cells of the wood, and then submitting the wood to a liquid preservative at a pressure substantially above atmospheric pressure to seal the cells of the wood.

2. The process of preserving wood which comprises submitting the wood to compressed air at a pressure substantially above atmospheric pressure, submitting the wood to the action of a liquid preservative at a pressure substantially above that of the compressed air thereby coating the walls of the interior cells of the wood with the preservative, submitting the wood to a vacuum pressure, and then submitting the wood to a liquid preservative at a pressure less than that at which the first preservative was applied to seal the cells of the wood.
3. The process of preserving wood which comprises submitting the wood to an atmosphere of compressed air at a pressure substantially above atmospheric pressure, submerging the wood in a liquid preservative at a pressure substantially above that of the atmosphere of compressed air, maintaining such pressure on the liquid preservative until a predetermined proportion of the total amount of preservative to be taken up by the wood has been absorbed thereby, then submitting the wood to a vacuum pressure at a sufficient pressure and for a sufficient period of time to remove air and surplus preservative from the wood, and then submerging the wood to a liquid preservative at a sufficient pressure and for a sufficient period of time to cause the wood to take up the remaining proportion of the total amount of preservative.
4. The process of preserving wood which comprises submitting the wood to compressed air at a pressure of at least 40 pounds per square inch, then submitting the wood, without releasing such compressed air pressure to a liquid preservative at a pressure of at least 150 pounds per square inch until a predetermined proportion of the total amount of the preservative to be taken up by the wood has penetrated the same, then submitting the wood to a vacuum pressure of about 15 inches of mercury for a period of at least 20 minutes, and then submitting the wood to a liquid preservative at a pressure of at least 110 pounds per square inch until the remaining proportion of the total amount of the preservative to be taken up by the wood has penetrated the same.

HERBERT D. HECKERT.